

## UNITED STATES PATENT OFFICE

2,668,127

METHOD OF MOTH PROOFING WOOLEN  
GOODS

Erik Birger Eriksson, Norrkoping, Sweden

No Drawing. Application August 28, 1951,  
Serial No. 244,106Claims priority, application Sweden  
September 1, 1950

2 Claims. (Cl. 117—55)

1

For many years it has been desired to protect, in the cheapest possible way, woollen articles, such as clothing and yarn, against attack of keratin eating insects, especially moth larvae. It has inter alia long been known that the presence of fluorine in woollen goods gives such protection, and a considerable number of different compounds of fluorine have been manufactured and sold as anti-moth preparations. In the case of water-soluble silico fluorides, however, it has not been heretofore possible to provide a deposit on the wool which is resistant to washing, and the production of these preparations is now-a-days more or less dropped because of this lack of washing fastness. The general opinion has been that a chemical combination between the silico fluorides and the wool is not at all possible, but only a mere impregnation with the water-soluble salt.

Investigations have now shown that the acid residues resulting from earlier treatments of the wool in acid baths and coupled to the amino groups of the wool are substantially responsible for the fact that the water-soluble silico fluorides will not be linked. It has been proved that the presence of even very small amounts of acid residues in the wool prevents the desired genuine fixation of the silico fluorides.

The present invention has for its object a method which makes possible such a fixation of the water-soluble silico fluorides to the wool. As these compounds, preferably ammonium and sodium silico fluoride, are very cheap salts in comparison to the usually employed anti-moth agents, it will be possible according to the invention to obtain an extensive and general protection of woollen fabrics against moth and other keratin eating insects. The method is characterized in that the wool before its treatment in a water-soluble silico fluoride bath is treated in an alkaline bath containing an excess of alkali and then rinsed in water, so that all the acid residues linked to the wool are effectively neutralized and removed.

When the wool is freed from acid residues by neutralization, preferably with ammonia but also with other alkaline agents, and rinsed it will be sufficient to obtain the desired fixation to treat it for a short period of time in a slightly acid bath of water-soluble silico fluoride at room

temperature. An increase of the temperature of the bath will only slightly increase the amount of fluoride absorbed by the wool. If desired, a further rinsing in water may take place before drying. The woollen material may then be subjected to repeated washings in water solutions as well as in fat dissolving agents (chemical cleaning) without disappearance of the protecting effect. This has been proved in the first place by subjecting the woollen material, according to standard methods, to the attack of maximally vigorous moth larvae and in the second place by analytical determination of the amount of fluorine in the wool before and after the washings.

The analytical determinations have shown that contrary to earlier experience the wool chemically absorbs considerable amounts of fluorine, and that some portion of this fluorine will be so firmly fixed to the woollen substance that after the first washing no more fluorine can be removed by repeated washings. Normal data of analysis of the content of fluorine in the unwashed material are 0.4—0.5%, while after repeated washings the fluorine content invariably is about 0.23—0.25%. When washing in organic solvents, such as trichloroethylene, no fluorine is removed whatsoever, depending on the insolubility of the silico fluorides in such solutions.

As mentioned above, the woollen substance absorbs silico fluoride from the bath when the conditions of treatment are the right ones. At a ratio of for instance 1:30 between woollen material and liquid, with an addition of 3% ammonium silico fluoride, calculated on the weight of the material, and after pressing out the solution to about 100 parts liquid to 100 parts material, the fluorine content should not after drying be greater than 0.1%, unless no chemical binding had occurred. However, in these tests the fluorine content amounted to 0.4—0.5% in spite of the fact that before drying the impregnated cloth had been further rinsed for 10 minutes in flowing water.

To achieve a fully satisfactory protection against moth the wool must contain at least 0.15% fluorine. At this content the moth larvae will be killed upon eating very small quantities of the wool, and the loss of weight of such a material is after the attack of moth larvae under

## 3

standardized testing conditions considerably lower than the amount of 0.8 mg. per larvae which is indicated as an acceptable limit for the attack of moth larvae on an entirely antimoth proofed woollen fabric.

In spite of deficient knowledge about the nature of the bonds between the silico fluorides and the wool it appears that it is not a question of genuine valence combinations, but a question of coordinative binding forces between the silico fluoride complex and the wool substance. These binding forces will be fully developed only when the amino groups of the wool substance are entirely free from acid residues, and consequently it is obvious that they will in the first place act between these amino groups and the silico fluorides. A blocking of the amino groups by anions from dye-stuffs to a normal, i. e. to a relatively limited, extent, does not seem to disturb the binding forces, but such a disturbance appears only when blocking occurs by acid anions which cause a decrease of the pH value in the surface layer of the fibres.

The susceptibility of the fibre material to acid is very great. Thus, experiments have shown that woollen material which has been subjected to treatment in an acid bath (dye bath), then carefully rinsed in water and further treated in a buffered solution having a pH value of 6, could not fix the silico fluorides in a subsequent treatment in a solution of silico fluoride having a normal pH value of 4.0 to 4.5, so that a washing fastness was obtained. Thus, in all such cases where acid residues are present in the wool a real neutralization with a small excess of alkali must be carried out to obtain a fixation resistant to washing. If the treatment with silico fluoride is carried out on a non-neutralized material a normal absorption of silico fluoride in the wool (0.4-0.5% fluorine) will generally be obtained, but the fixation will not be genuine and most of the fluorine will be removed upon ordinary washing. Neutralization with ammonium is to be preferred as it will then be easier to remove the excess of alkali by rinsing than if soda is used.

Besides being resistant to alkaline washing the bond between a neutral wool and silico fluoride is to a certain extent intact also against the action of a boiling acid bath. If the concentration of the acid is increased to such an extent that the pH value falls below 3.0, the bond will gradually break up, so that the fluorine is removed. This means that in such cases where it is a question of dyeing wool free from acid in a dye bath not containing great quantities of acid (acid dyeing or chrom dyeing) the treatment with silico fluoride may take place just before the dyeing.

It has also been proved that a neutral wool can be treated in a silico fluoride bath to which considerable amounts of acid have been added and a resistant fixation of the silico fluoride in the wool may be obtained. In this case it appears that the silico fluoride is bound to the wool so quickly that a reaction between the acid and the amino groups of the wool will not have time to occur to any noticeable degree until the silico fluorides are already fixed. Thus, when it is the question of dyeing wool free from acid in a dye bath containing small quantities of acid (1.0-2.0% of the weight of the wool) it is in practice possible to carry out the treatment with silico fluoride at the same time as the dyeing. When on the other hand the dyeing bath contains greater amounts of acid (neulan-dyeing) the treatment with silico fluoride can be carried out

## 4

only after the dyeing and must then be preceded by a careful neutralization. In this connection it will be observed that a so-called carbonization after a treatment with silico fluoride entirely destroys the anti-moth protecting effect in that the silico fluoride is destroyed and decomposed by the concentrated sulphuric acid which in this process acts on the wool during the drying. After neutralization of the acid woollen material it is, however, possible to treat the material successfully with silico fluoride in a normal way.

It has furthermore been found that the fixation effect is further improved if the wool after the treatment with silico fluoride is treated in a bath containing ordinary soaps of fatty acids. Certainly, the fixation effect obtained by the method described above is sufficient to prevent the silico fluorides from being removed by a simple rinsing in water, and as soon as the cloth is washed in a soap solution the above-mentioned complete fixation will take place. If, however, the washings are instead carried out by means of synthetic washing agents it has been shown that the silico fluorides are extracted to a large extent, and it may therefore be necessary to carry out a complete fixation of the silico fluoride in the factory by a simple treatment in soap solution. After such treatment the following washings in synthetic washing agents will cause no noticeable extraction of fluoride.

Regarding the nature of the fixation achieved in this way nothing can be said with certainty but conditions are likely to be the following. Only a part of the amino groups of the wool are responsible for the genuine fixation of the silico fluorides. These amino groups are evidently very easily blocked by acids which is why the wool must be neutralized before the silico fluoride treatment, which should be carried out at a pH value about corresponding to the natural pH value of the acid ammonium silico fluoride solutions. If these amino groups are free they will in the first place form salts with the silico fluorides. In the subsequent treatment with soap small amounts of fatty acids are likely to be precipitated as the wool is acid. On account of special relations between adjacent polar groups the precipitated fatty acids will evidently enter into some complex formation between the wool and the silico fluorides. The cloth thus impregnated with silico fluoride and treated with soap may then be subjected to repeated washings in alkaline baths as well as in baths containing different kinds of synthetic washing agents without the silico fluoride being removed but to the limit (about 0.20% fluorine based on the weight of the wool) determined by the active groups in the wool.

## Example 1

A strip of white woollen fabric weighing 30 g. was dyed by boiling for 2 hours with 3% neulan-dyestuff (neulan red GRE) in a dye bath containing 8% sulphuric acid and 10% crystallized sodium sulphate, calculated on the weight of the fabric. The fabric was rinsed in flowing water during 30 min. and then treated for 10 min. at room temperature in a solution containing 0.05-normal ammonia at a ratio of 1:25 between material and liquid. The material was then rinsed for 5 min. in flowing water and treated for 20 min. at a temperature of about 25° C. in a solution containing 3% ammonium silico fluoride, calculated on the weight of the material at a bath ratio of 1:25. Finally rinsing

5

in flowing water for 10 min. and drying took place.

For determination of the washing fastness of the impregnation, samples of the impregnated fabric were washed 1, 2 and 4 times respectively in a solution containing 5 g. soap per liter. The treatment took place during half an hour at a bath ratio of 1:50 and a temperature of 40° C. After each washing the fabric was rinsed 3 times for 2 min. each time in distilled water at 40° C. In biological testing with moth larvae and in analyzing the amount of fluorine in the fabric the results in the following table were obtained:

| Fabric              | Consumption in mg./larvae | Percent fluorine in the fabric |
|---------------------|---------------------------|--------------------------------|
| Unwashed.....       | 0.20                      | 0.45                           |
| Washed once.....    | 0.47                      | 0.23                           |
| Washed twice.....   | 0.49                      | 0.22                           |
| Washed 4 times..... | 0.50                      | 0.22                           |

#### Example 2

A strip of chromium-dyed and carbonized but not fully neutralized woollen fabric containing 1.2% sulphuric acid was treated for 15 min. at room temperature in a 0.05-normal solution of soda at a bath ratio of 1:25. The fabric was rinsed in flowing water for 15 min. and treated at 25° C. for 20 min. at a bath ratio of 1:25 in a solution containing 3% ammonium silico fluoride, calculated on the weight of the fabric. Finally, the fabric was rinsed in flowing water for 10 min.

In biological testing with moth larvae and in analyzing the amount of fluorine the results in the following table were obtained. The washings of the samples were carried out as in Example 1:

| Fabric              | Consumption in mg./larvae | Percent fluorine in the fabric |
|---------------------|---------------------------|--------------------------------|
| Unwashed.....       | 0.23                      | 0.47                           |
| Washed once.....    | 0.54                      | 0.21                           |
| Washed twice.....   | 0.56                      | 0.20                           |
| Washed 4 times..... | 0.56                      | 0.20                           |

#### Example 3

A strip of undyed but carbonized and not fully neutralized woollen fabric was treated for 15 min. at room temperature in a 0.05-normal ammonia solution at a bath ratio of 1:25. The fabric was then rinsed in flowing water for 15 min. and treated at 25° C. for 20 min. at a bath ratio of 1:25 in a solution containing 3% ammonium silico fluoride, calculated on the weight of the fabric. 3% sulphuric acid, 10% crystallized sodium sulphate and 3% Azorhodin 2G was then added to the ammonium silico fluoride bath, whereupon dyeing took place by increasing the temperature to 100% C. and boiling for 1 hour.

Finally, the fabric was rinsed in flowing water for  $\frac{1}{2}$  hour. In biological testing with moth larvae and in analyzing the amount of fluorine the results in the following table were obtained. The washings of the samples were carried out as in Example 1:

| Fabric              | Consumption in mg./larvae | Percent fluorine in the fabric |
|---------------------|---------------------------|--------------------------------|
| Unwashed.....       | 0.30                      | 0.40                           |
| Washed once.....    | 0.61                      | 0.20                           |
| Washed twice.....   | 0.63                      | 0.19                           |
| Washed 4 times..... | 0.65                      | 0.19                           |

6

#### Example 4

20 g. white uncarded wool was dyed by boiling for 1 hour with 3% Azorhodin 2G in a dye bath containing 3% sulphuric acid and 10% crystallized sodium sulphate, calculated on the weight of the wool. The wool was then rinsed in flowing water for 30 min. and treated at room temperature for 10 min. in a solution containing 0.05-normal ammonia at a bath ratio of 1:50. The wool was rinsed for 10 min. in flowing water and treated for 10 min. at a temperature of about 25° C. in a solution containing 3% ammonium silico fluoride, calculated on the weight of the wool, at a bath ratio of 1:50. Finally, rinsing in flowing water for 10 min. and drying took place.

In biological testing with moth larvae and in analyzing the amount of fluorine the results in the following table were obtained. The washings of the samples were carried out as in Example 1:

| Fabric              | Consumption in mg./larvae | Percent fluorine in the wool |
|---------------------|---------------------------|------------------------------|
| Unwashed.....       | 0.20                      | 0.45                         |
| Washed once.....    | 0.43                      | 0.24                         |
| Washed twice.....   | 0.46                      | 0.22                         |
| Washed 4 times..... | 0.49                      | 0.22                         |

#### Example 5

A white woollen fabric was neutralized with ammonia and rinsed in flowing water. The fabric was then impregnated at a temperature of 25° C. and a bath ratio of 1:25 for 20 min. in an ammonium silico fluoride solution of varying concentration. Finally, the fabric was rinsed in flowing water of room temperature for 20 min. The results are given in the following table. The amount of silico fluoride is given in percentage of weight of the fabric.

| Content of ammonium silico fluoride in the bath in percent of weight of fabric | Unwashed | Washed once | Washed twice |
|--------------------------------------------------------------------------------|----------|-------------|--------------|
| 1.....                                                                         | 0.25     | 0.19        | 0.18         |
| 2.....                                                                         | 0.32     | 0.21        | 0.21         |
| 3.....                                                                         | 0.39     | 0.21        | 0.20         |
| 4.....                                                                         | 0.40     | 0.21        | 0.21         |
| 5.....                                                                         | 0.43     | 0.21        | 0.20         |

The results show in the first place that it is sufficient to use as small quantity of silico fluoride as 1% of weight of the fabric. It is furthermore evident that the wool is capable of binding about 0.20% fluorine disregarding the concentration of silico fluoride in the bath. This is vigorous proof of the theory that a well neutralized wool will to a certain extent strongly bind silico fluoride and that the wool shows certain spots at which linkage may take place.

#### Example 6

Uncolored woollen cloth was treated with 0.05-n ammonia solution for 30 min., whereupon the cloth was rinsed in flowing water for 15 min. and then treated in a silico fluoride bath. The cloth was then divided into three parts which were further treated as follows:

1. One sample was washed four times (each time for 30 min.) at 40° C. in a solution containing 5 g./l. soap flakes.
2. One sample was washed four times in the same way in a solution containing 2 g./l. lauryl alcohol sulphonate.
3. One sample was first treated for 15 min. at

40° C. in a solution containing 3 g./l. soap, rinsed and washed four times in a solution containing 2 g./l. lauryl alcohol sulphonate. The results appear in the following table:

| Sample | Treatment                                        | Percent fluorine |
|--------|--------------------------------------------------|------------------|
| 1      | Unwashed.....                                    | 0.42             |
|        | Washed once in soap solution.....                | 0.22             |
|        | Washed twice in soap solution.....               | 0.20             |
|        | Washed four times in soap solution.....          | 0.20             |
| 2      | Unwashed.....                                    | 0.42             |
|        | Washed once in lauryl alcohol sulphonate.....    | 0.14             |
|        | Washed twice in lauryl alcohol sulphonate.....   | 0.10             |
|        | Washed 4 times in lauryl alcohol sulphonate..... | 0.09             |
| 3      | Washed once in soap solution.....                | 0.25             |
|        | Washed once in lauryl alcohol sulphonate.....    | 0.22             |
|        | Washed twice in lauryl alcohol sulphonate.....   | 0.21             |
|        | Washed 4 times in lauryl alcohol sulphonate..... | 0.21             |

Test No. 3 proves that about 0.20% fluorine is fixed to the wool by the soap treatment, so that thereafter extraction by washing does not occur.

*Example 7*

A colored woollen cloth was neutralized as in Example 6 with ammonia, rinsed in flowing water for 15 min. and treated with silico fluoride. The cloth was divided into two parts, one of which was treated at room temperature for 30 min. in a solution containing 5 g./l. soap and then rinsed, while the other one was not subjected to such treatment. Both samples were put in distilled water, which was changed every day. Analysis of the fluorine content in each piece of cloth was made after different periods of extraction in distilled water. The results appear in the following table:

| Time in water | Percent fluorine      |                   |
|---------------|-----------------------|-------------------|
|               | Not treated with soap | Treated with soap |
| 2 days.....   | 0.43                  | 0.25              |
| 5 days.....   | 0.39                  | 0.24              |
| 7 days.....   | 0.29                  | 0.24              |
| 12 days.....  | 0.22                  | 0.24              |
| 17 days.....  | 0.10                  | 0.23              |
| 20 days.....  | 0.07                  | 0.23              |
|               | 0.04                  | 0.23              |

The table shows that a good fixation is achieved by the treatment with soap.

I claim:

5 1. A method of moth proofing woolen goods containing acid residues deposited in said goods during the manufacture thereof, which comprises treating the woolen goods in a water solution containing an alkaline neutralizing agent in an amount in excess of that required to neutralize 10 all of said acid residues in the woolen goods, rinsing the woolen goods in water to remove the neutralized acid residues, immersing the wool in a water solution containing a water-soluble silico fluoride in an amount corresponding to at least about 1% by weight of the goods, and drying the woolen goods, whereby said fluoride becomes firmly fixed to the fibers of said woolen goods and is resistant to displacement therefrom upon repeated washing.

20 2. A method of moth proofing woolen goods as defined in claim 1, further comprising the step of immersing the woolen goods after immersion in the water solution of the silico fluoride in a water solution containing a water-soluble fatty acid soap.

ERIK BIRGER ERIKSSON.

References Cited in the file of this patent

UNITED STATES PATENTS

| Number    | Name           | Date          |
|-----------|----------------|---------------|
| 1,634,790 | Minaeff .....  | July 5, 1927  |
| 1,682,975 | Meckbach ..... | Sept. 4, 1928 |
| 1,914,059 | White .....    | June 13, 1933 |